



US006849379B2

(12) **United States Patent**  
**Oohashi et al.**

(10) **Patent No.:** **US 6,849,379 B2**  
(45) **Date of Patent:** **Feb. 1, 2005**

(54) **LITHOGRAPHIC PRINTING PLATE  
PRECURSOR**

(75) Inventors: **Hidekazu Oohashi**, Shizuoka (JP);  
**Shinnichi Morishima**, Kanagawa (JP)

(73) Assignee: **Fuji Photo Film Co., Ltd.**, Kanagawa (JP)

(\*) Notice: Subject to any disclaimer, the term of this patent is extended or adjusted under 35 U.S.C. 154(b) by 0 days.

(21) Appl. No.: **10/262,065**

(22) Filed: **Oct. 2, 2002**

(65) **Prior Publication Data**

US 2003/0129522 A1 Jul. 10, 2003

(30) **Foreign Application Priority Data**

Oct. 3, 2001 (JP) ..... P. 2001-307616

(51) **Int. Cl.<sup>7</sup>** ..... **G03F 7/004**

(52) **U.S. Cl.** ..... **430/270.1**; 430/138; 430/273.1;  
430/302; 430/309; 430/348

(58) **Field of Search** ..... 430/138, 270.1,  
430/271.1, 273.1, 302, 309, 348

(56) **References Cited**

U.S. PATENT DOCUMENTS

3,628,953 A \* 12/1971 Brinckman ..... 430/325

4,004,924 A \* 1/1977 Vrancken et al. ..... 430/325  
6,225,024 B1 \* 5/2001 Morishima et al. .... 430/270.18  
6,558,880 B1 \* 5/2003 Goswami et al. ..... 430/350  
6,573,022 B1 \* 6/2003 Miyake et al. ..... 430/270.1  
6,579,662 B1 \* 6/2003 Zheng et al. ..... 430/281.1  
6,646,132 B2 \* 11/2003 Morishima et al. ..... 546/347  
2002/0009669 A1 \* 1/2002 Morishima et al. .... 430/270.18  
2002/0081522 A1 \* 6/2002 Miyake et al. ..... 430/270.1  
2003/0064205 A1 \* 4/2003 Morishima et al. ..... 428/195  
2003/0091932 A1 \* 5/2003 Loccufier et al. ..... 430/272.1

FOREIGN PATENT DOCUMENTS

|    |            |   |         |       |           |
|----|------------|---|---------|-------|-----------|
| EP | 962 923 A1 | * | 12/1999 | ..... | G11B/7/24 |
| JP | 10-337962  |   | 12/1998 |       |           |
| JP | 11-277927  |   | 10/1999 |       |           |
| JP | 2001-33953 |   | 2/2001  |       |           |

\* cited by examiner

Primary Examiner—Barbara L. Gilliam

(74) Attorney, Agent, or Firm—Sughrue Mion, PLLC

(57) **ABSTRACT**

A lithographic printing plate precursor having an image-forming layer capable of drawing images by heat or heat mode exposure, which comprises a support and a layer containing a heat decomposable dye having an absorption maximum wavelength in a visible region, not substantially having an absorption in an oscillation wavelength of a laser used for heat mode exposure, and having a heat decomposition initiation temperature of 250° C. or lower.

**11 Claims, No Drawings**

**1**  
**LITHOGRAPHIC PRINTING PLATE  
PRECURSOR**

**FIELD OF THE INVENTION**

The present invention relates to a lithographic printing plate precursor capable of drawing images by heat or heat mode exposure, in particular, to a lithographic printing plate precursor forming printout images that can be visibly confirmed with ease after drawing the images by heat or heat mode exposure.

**BACKGROUND OF THE INVENTION**

Hitherto, the preparation of printing plates for lithographic printing has been carried out in a system in which a printing plate precursor is exposed to light through a lith film as an intermediate material. However, in recent years, as the digitalization rapidly proceeds in the printing field, the preparation step of the printing plate is being changed to a computer-to-plate (CTP) system in which digital data input and edited in a computer are directly output to a printing plate precursor. As the printing plate precursor for CTP, are proposed various modes as described, for example, in *Journal of Printing Science and Technology*, Vol. 36, pp. 97-104 and pp. 148-163 (1999). Of these are also actively studied lithographic printing plate precursors capable of drawing images by heat or heat mode exposure.

Even in such a lithographic printing plate precursor capable of drawing images by heat or heat mode exposure, like in conventional lithographic printing plate precursors, it is important in the printing plate preparation work to discriminate whether or not the precursor is already exposed to light, to inspect images on the printing plate, and to distinguish the plate to which what color of inks should be applied. In particular, since development is not carried out in a printing plate requiring no development, inspection and discrimination of the plate are difficult in mounting the plate on a printing press, and hence, a method for compensating these difficulties is required.

To solve such difficulties, JP-A-11-2717927 (the term "JP-A" as used herein means an "unexamined published Japanese patent application") describes a printing plate comprising, on a support, a recording layer containing a light-heat converting agent, a compound generating an acid, a base or a radical by light or heat, and a compound that discolors by a mutual action with the generated acid, base or radical, which can be exposed with an infrared laser and has exposed image-visualizing property (printout property).

However, the compound generating an acid or a radical, which is suitable for obtaining a printout image as described in the above patent, has an absorption in a visible light region. Accordingly, in the printing plate using such a compound, the acid or radical is generated during standing in a light room before or after the imagewise exposure, to cause discoloration. As a result, there are involved problems such that the generation of the printout image during imagewise exposure is inhibited and that the generated printout image becomes unclear during a time when the plate exposed imagewise is allowed to stand.

JP-A-2001-33953 describes that in a light-sensitive material comprising, on a support, a recording layer containing an electron-accepting polymer soluble in an alkaline developing solution and a near infrared-absorptive dye, when near infrared light is irradiated, the optical reflection density in the irradiated area of the recording layer decreases so that drawn images can be visually confirmed at the time of

completion of the exposure. However, the dye used in the technology is an electron-donating dye precursor, from which a readily visual printout image can be obtained only in the presence of the electron-accepting polymer, and hence, such a dye is not a general-purpose dye for printout.

**SUMMARY OF THE INVENTION**

An object of the invention is to provide a lithographic printing plate precursor having good printout property, which can overcome the above-described problems and is capable of drawing images by heat or heat mode exposure. Another object of the invention is to provide a lithographic printing plate precursor having good printout property and capable of being subjected to printing without processing such as development, after drawing images.

The present inventors have been able to achieve the above-described objects by using a heat decomposable dye having an absorption maximum wavelength in a visible region and not substantially having an absorption in an oscillation wavelength of a laser used for heat mode exposure. Specifically, the invention includes the following lithographic printing plate precursors.

1. A lithographic printing plate precursor having an image-forming layer capable of drawing images by heat or heat mode exposure, which comprises a support and a layer containing a heat decomposable dye having an absorption maximum wavelength in a visible region, not substantially having an absorption in an oscillation wavelength of a laser used for heat mode exposure, and having a heat decomposition initiation temperature of 250°C. or lower.
2. The lithographic printing plate precursor as described in item 1 above, wherein the lithographic printing plate precursor is a lithographic printing plate precursor that can be mounted directly on a printing press without a development processing after exposure.
3. The lithographic printing plate precursor as described in item 1 or 2 above, wherein the heat decomposable dye has a structure represented by the following formula (1) or (2):



wherein, A, A', B, and B' each independently represents a substituent; Y and Z each represents an atomic group necessary for forming a carbon ring or a heterocyclic ring; E and G each represents an atomic group to complete a conjugated double bond chain; X and X' each represents oxygen, N—R, or C(CN); R represents an alkyl group or an aryl group; L<sup>3</sup>, L<sup>4</sup>, L<sup>5</sup>, L<sup>6</sup>, and L<sup>7</sup> each represents a methine group which may be substituted; M<sup>k+</sup> represents an onium ion; m and n each independently represents 0, 1, or 2; x and y each independently represents 0 or 1; and k represents an integer of 1 or more.

4. The lithographic printing plate precursor as described in item 1 above, wherein the image-forming layer comprises

- a hydrophobic polymer compound that can be rendered hydrophilic by heat and has a functional group selected from a sulfonic ester group, a sulfonimido group and a disulfone group.
5. The lithographic printing plate precursor as described in item 1 above, wherein the image-forming layer comprises fine particles of a thermoplastic hydrophobic polymer.
  6. The lithographic printing plate precursor as described in item 1 above, wherein the image-forming layer comprises microcapsules encapsulating an oleophilic compound.
  7. The lithographic printing plate precursor as described in item 1 above, wherein the lithographic printing plate precursor is a lithographic printing plate precursor comprising a hydrophilic layer provided on an oleophilic layer, which is subjected to heat mode laser exposure to remove imagewise the hydrophilic layer by ablation, thereby forming images.

#### DETAILED DESCRIPTION OF THE INVENTION

In the invention, in order to obtain printout images, is used a heat decomposable dye having an absorption maximum wavelength in a visible region, not substantially having an absorption in an oscillation wavelength of a laser used for heat mode exposure, and having a heat decomposition initiation temperature of 250° C. or lower. Since the dye is insensitive to a visible light, there is no problem of occurrence of fogging during handling in a light room. Further, the invention is not restricted with respect to a combination of an electron-donating dye precursor with an electron-accepting polymer, which is essential in the conventional technology for the purpose of obtaining good printout images, but can provide good printout images through any combination with polymers.

JP-A-10-337962 describes a heat-sensitive recording material comprising, on a support, a recording layer containing a ultraviolet-absorptive substance having a maximum absorption at from 330 to 430 nm or a dye having an absorption maximum in a visible region, and an infrared-absorptive substance to lower the maximum absorption intensity of the ultraviolet-absorptive substance or dye upon irradiation with a laser having an oscillation wavelength within the range of from 750 to 900 nm. In the heat-sensitive recording material, what the maximum absorption intensity of the ultraviolet-absorptive substance or dye is lowered upon irradiation with a laser is estimated to be caused by the matter that a redox reaction occurs between the infrared-absorptive substance and the ultraviolet-absorptive substance, or between the infrared-absorptive substance and the dye, at high temperature upon heating within a short period of time, whereby the ultraviolet-absorptive substance or the dye is decomposed. Also, the heat-sensitive recording material is aimed to form a negative used for contact exposure to a PS plate or a photomask, and the above-cited patent does not describe a lithographic printing plate. Accordingly, this technology does not at all disclose or even suggest the dissolution of the above-described problems as in the invention, in which printout property is imparted to the lithographic printing plate precursor using a heat decomposable dye that is decomposed singly by heat.

The invention will be described in more detail below.

The heat decomposable dye, which is used in the lithographic printing plate precursor according to the invention, is a dye having an absorption maximum wavelength in a visible region, not substantially having an absorption in an oscillation wavelength of a laser used for heat mode

exposure, and having a heat decomposition initiation temperature of 250° C. or lower. The dye not substantially having an absorption in an oscillation wavelength of a laser used for heat mode exposure means a dye that makes it impossible to form printout images, when a light-heat converting agent is removed from a layer containing the heat decomposable dye or a layer adjacent thereto. Namely, in the case of heat mode exposure, the heat decomposable dye used in the invention absorbs a heat generated by the light-heat converting agent to cause decomposition.

The heat decomposable dye that is used in the lithographic printing plate precursor according to the invention is subjected to heat decomposition to exhibit a hue different from that before the decomposition. By such change in the hue, a difference in the hue is generated between image areas and non-image areas of an image-forming layer, whereby it becomes easy to confirm the drawn images. Therefore, good printout images are obtained by using any polymer in the image-forming layer.

20 The heat decomposition initiation temperature of the heat decomposable dye used in the invention means a temperature at which the start of weight reduction or heat absorption/generation caused by the heat decomposition is observed, when the dye is measured at a temperature elevation rate of 10° C./min by means of a TG-DTA measurement device.

25 Although any dye can be used as the heat decomposable dye used in the lithographic printing plate precursor according to the invention so far as it meets the above-described requirements, dyes represented by the following formula (1) or (2) are particularly preferable.



35 wherein, A, A', B, and B' each independently represents a substituent; Y and Z each represents an atomic group necessary for forming a carbon ring or a heterocyclic ring; E and G each represents an atomic group to complete a conjugated double bond chain; X and X' each represents oxygen, N—R, or C(CN)<sub>2</sub>; R represents an alkyl group or an aryl group; L<sup>3</sup>, L<sup>4</sup>, L<sup>5</sup>, L<sup>6</sup>, and L<sup>7</sup> each represents a methine group which may be substituted; M<sup>k+</sup> represents an onium ion; m and n each independently represents 0, 1, or 2; x and y each independently represents 0 or 1; and k represents an integer of 1 or more.

40 Examples of the substituent represented by A, A', B or B' include a substituted or unsubstituted, linear, branched or cyclic alkyl group having from 1 to 18 carbon atoms, and preferably from 1 to 8 carbon atoms (such as methyl, ethyl, propyl, isopropyl, n-butyl, isobutyl, sec-butyl, tert-butyl, cyclohexyl, methoxyethyl, ethoxycarbonyethyl, cyanoethyl, diethylaminoethyl, hydroxyethyl, chloroethyl, and acetoxyethyl); a substituted or unsubstituted aralkyl group having from 7 to 18 carbon atoms, and preferably from 7 to 12 carbon atoms (such as benzyl and carboxybenzyl); an alkenyl group having from 2 to 18

carbon atoms, and preferably from 2 to 8 carbon atoms (such as vinyl); an alkynyl group having from 2 to 18 carbon atoms, and preferably from 2 to 8 carbon atoms (such as ethynyl); a substituted or unsubstituted aryl group having from 6 to 18 carbon atoms, and preferably from 6 to 10 carbon atoms (such as phenyl, 4-methylphenyl, 4-methoxyphenyl, 4-carboxyphenyl, and 3,5-dicarboxyphenyl); a substituted or unsubstituted acyl group having from 2 to 18 carbon atoms, and preferably from 2 to 8 carbon atoms (such as acetyl, propionyl, butanoyl, and chloroacetyl); a substituted or unsubstituted sulfonyl group having from 1 to 18 carbon atoms, and preferably from 1 to 8 carbon atoms (such as methanesulfonyl and p-toluenesulfonyl); a sulfinyl group having from 1 to 18 carbon atoms, and preferably from 1 to 8 carbon atoms (such as methanesulfinyl, ethanesulfinyl, and octanesulfinyl); an alkoxy carbonyl group having from 2 to 18 carbon atoms, and preferably from 2 to 8 carbon atoms (such as methoxy carbonyl and ethoxycarbonyl); an aryloxycarbonyl group having from 7 to 18 carbon atoms, and preferably from 7 to 12 carbon atoms (such as phenoxy carbonyl, 4-methylphenoxy carbonyl, and 4-methoxyphenoxy carbonyl); a substituted or unsubstituted alkoxy group having from 1 to 18 carbon atoms, and preferably from 1 to 8 carbon atoms (such as methoxy, ethoxy, n-butoxy, and methoxyethoxy); a substituted or unsubstituted aryloxy group having from 6 to 18 carbon atoms, and preferably from 6 to 10 carbon atoms (such as phenoxy and 4-methoxyphenoxy); an alkylthio group having from 1 to 18 carbon atoms, and preferably from 1 to 8 carbon atoms (such as methylthio and ethylthio); an arylthio group having from 6 to 10 carbon atoms (such as phenylthio); a substituted or unsubstituted acyloxy group having from 2 to 18 carbon atoms, and preferably from 2 to 8 carbon atoms (such as acetoxy, ethylcarbonyloxy, cyclohexylcarbonyloxy, benzyloxy, and chloroacetyloxy); a substituted or unsubstituted sulfonyloxy group having from 1 to 18 carbon atoms, and preferably from 1 to 8 carbon atoms (such as methanesulfonyloxy); a carbamoyloxy group having from 2 to 18 carbon atoms, and preferably from 2 to 8 carbon atoms (such as methylcarbamoyloxy and diethylcarbamoyloxy); a substituted or unsubstituted amino group having from 0 to 18 carbon atoms, and preferably from 0 to 8 carbon atoms (such as unsubstituted amino, methylamino, dimethylamino, diethylamino, anilino, methoxyphenylamino, chlorophenylamino, morpholino, piperidino, pyrrolidino, pyridylamino, methoxycarbonylamino, n-butoxycarbonylamino, phenoxy carbonylamino, methylcarbamoylamino, phenylcarbamoylamino, ethylthiocarbamoylamino, methylsulfamoylamino, phenylsulfamoylamino, acetyl amino, ethylcarbonylamino, ethylthiocarbonylamino, cyclohexylcarbonylamino, benzyloxy, chloroacetyl amino, methanesulfonylamino, and benzenesulfonylamino); a substituted or unsubstituted carbamoyl group having from 1 to 18 carbon atoms, and preferably from 1 to 8 carbon atoms (such as unsubstituted carbamoyl, methylcarbamoyl, ethylcarbamoyl, n-butylcarbamoyl, tert-butylcarbamoyl, dimethylcarbamoyl, morpholinocarbamoyl, and pyrrolidinocarbamoyl); a substituted or unsubstituted sulfamoyl group having from 0 to 18 carbon atoms, and preferably from 0 to 8 carbon atoms (such as unsubstituted sulfamoyl, methylsulfamoyl, and phenylsulfamoyl); a halogen atom (such as fluorine, chlorine, and bromine); a hydroxy group; a nitro group; a cyano group; a carboxyl group; and a heterocyclic group (such as oxazole, benzoxazole, thiazole, benzothiazole,

imidazole, benzimidazole, indolenine, pyridine, sulfolane, furan, thiophene, pyrazole, pyrrole, chroman, and coumarin).

As the substituent represented by A or A' are preferable those having a Hammett's substituent constant,  $\sigma_p$  value of 0.2 or more. The Hammett's substituent constant is described, for example, in *Chem. Rev.*, Vol. 91, 165(1991). Particularly preferred examples of the substituent include a cyano group, a nitro group, an alkoxy carbonyl group, an acyl group, a carbamoyl group, a sulfamoyl group, and a sulfonyl group.

As the substituent represented by B or B' are preferable an alkyl group, an aryl group, an alkoxy group, and an amino group.

Since  $—C—(E)_x—C(=X)—$  bonding to Y and  $—C(=G)_y—C(=X')—$  bonding to Z are in a conjugated state with each other, the carbocyclic ring or heterocyclic ring represented Y and  $—C—(E)_x—C(=X)—$  bonding to Y, and the carbocyclic ring or heterocyclic ring represented by Z and  $—C(=G)_y—C(=X')—$  bonding to Z may be respectively considered as one of resonance structures. The carbocyclic ring or heterocyclic ring is hereinafter referred to as a carbocyclic ring or heterocyclic ring represented by Y and Z, and  $—C—[(E)_x \text{ and } (G)_y]—C(=X \text{ and } X')—$  bonding thereto for the sake of convenience. As the carbocyclic ring or heterocyclic ring represented by Y and Z, and  $—C—[(E)_x \text{ and } (G)_y]—C(=X \text{ and } X')—$  bonding thereto are preferable 4-membered, 5-membered, 6-membered, and 7-membered rings, with the 5-membered and 6-membered rings being particularly preferred. These rings may be further taken together with other 4-membered, 5-membered, 6-membered, or 7-membered ring to form a fused ring. These rings may have a substituent. As the substituent are employable those as enumerated above for A, A', B, and B'. As a hetero atom forming the heterocyclic ring are preferable B, N, O, S, Se, and Te, with N, O, and S being particularly preferred. x and y each independently represents 0 or 1, and preferably 0.

X and X' each represents any one of oxygen, N—R, and C(CN)<sub>2</sub>, and preferably oxygen. Examples of the carbocyclic ring formed by Y and Z, and  $—C—[(E)_x \text{ and } (G)_y]—C(=X \text{ and } X')—$  bonding thereto are enumerated below.

BB-1



BB-2



BB-3



7

-continued



5

BB-4

8

-continued



BB-12

BB-13



BB-14



BB-15



BB-16



BB-17



BB-18



BB-19



BB-20



Of these carbocyclic rings are preferable BB-1 and BB-4.

Examples of the heterocyclic ring formed by Y and Z, and —C—[(E)<sub>x</sub> and (G)<sub>y</sub>]—C(=X and X')— bonding thereto are enumerated below:



BB-5

20



BB-6

25



BB-7

30



BB-8

40



BB-9

45



BB-10

50



BB-11

60

65



11

-continued



BB-39

5

BB-40

10

BB-41

15



20

(1)



30



(2)



45



(3)



(4)

Of these heterocyclic rings are preferable BB-5, BB-6, 25  
BB-7, BB-11, BB-14, and BB-39.

Ra, Rb, and Rc each independently represents a hydrogen atom or a substituent. The substituent represented by Ra, Rb, or Rc has the same meaning as the substituent represented by A, A', B, and B', or the substituents are connected to each other to form a ring. Examples of the ring formed include a cyclohexane ring and a benzene ring.

The methine groups represented by L<sup>3</sup>, L<sup>4</sup>, L<sup>5</sup>, L<sup>6</sup>, and L<sup>7</sup> may be the same or different and may have a substituent. The substituent has the same meaning as the substituent represented by each of A, A', B, and B'. Preferred examples of the substituent include an alkyl group, an aralkyl group, an aryl group, an alkoxy group, an aryloxy group, an alkylthio group, an arylthio group, a halogen atom, an amino group, a carbamoyl group, and a heterocyclic group. Also, the substituents may be connected to each other to form a 35 5-membered, 6-membered, or 7-membered ring (such as cyclopentene ring, 1-dimethylaminocyclopentene ring, 1-diphenylaminocyclopentene ring, cyclohexene ring, 1-chlorocyclohexene ring, isophorone ring, 40 1-morpholinocyclohexene ring, and cycloheptene ring).

Examples of the onium ion represented by M<sup>k+</sup> include an alkali metal ion (such as a sodium ion, a potassium ion, and a lithium ion), an ammonium ion, an anilinium ion, a quaternary ammonium ion, an oxonium ion, a sulfonium ion, a phosphonium ion, a selenonium ion, and an iodonium 45 50 ion. It is preferred that M<sup>k+</sup> is not a cyanine dye.

The quaternary ammonium ion is generally obtained by alkylating, alkenylating, alkynylating, or arylating a tertiary amine (such as trimethylamine, triethylamine, tributylamine, triethanolamine, N-methylpyrrolidine, 55 N-methylpiperidine, N,N-dimethylpiperazine, triethylenediamine, and N,N,N',N'-tetramethylenediamine) or a nitrogen-containing heterocyclic compound (such as pyridine, picoline, 2,2'-bipyridyl, 4,4'-bipyridyl, 1,10-phenanthroline, quinoline, oxazole, thiazole, 60 N-alkylimidazole, N-alkylbenzimidazole, pyrazine, tetrazole, N-alkylpiperidine, and N-alkylmorpholine).

k represents an integer, preferably from 1 to 20, more preferably from 1 to 4, and particularly preferably 2.

The dye represented by the foregoing formula (1) or (2) 65 can be synthesized according to the method as described in JP-A-10-109476 or JP-A-2000-52658.

12

Specific examples of the heat decomposable dye that is used in the invention are described below, but the invention should not be construed as being limited thereto.

5

(1)



15



(2)



30



(3)



45



(4)



**13**

-continued



5



(5)

15



20



(6)

30



35

40

45



50

55



60

65

**14**

-continued

(9)



(10)



(11)



(12)



(13)



15

-continued



A printout element using the heat decomposable dye according to the invention can be applied to various lithographic printing plate precursors capable of drawing images by heat or heat mode exposure. Examples of the applicable lithographic printing plate precursors include those described below.

- (1) A CTP lithographic printing plate precursor free from development processing, which is provided with a polarity-converting material-based image-forming layer containing an oleophilic polymer having a specified sulfonimidoo group, disulfone group or sulfonic ester group on the side chains thereof, the oleophilic polymer being converted into a sulfonic acid-containing hydrophilic polymer by heat and/or an acid, as described in JP-A-10-282642, JP-A-10-282644, JP-A-10-282646, and JP-A-10-282672.
- (2) A CTP lithographic printing plate precursor free from development processing, which uses a polymer polarity-converting material containing a group selected from decarboxylation-causing carboxylic acid groups such as an  $\alpha$ -sulfonylacetic acid structure and carboxylic acid salt groups, as described in JP-A-2000-122272.
- (3) A positive type heat-sensitive lithographic printing plate precursor utilizing a phenomenon in which when a heat is applied to an associative polymer such as novolak resin, solubility increases, a difference in the solubility from that in areas to which the heat is not applied is caused, and development with an aqueous alkaline solution is carried out to form a positive image, as described, for example, in JP-B-46-27919 and JP-A-7-285275.
- (4) A negative type heat-sensitive lithographic printing plate precursor having a heat crosslinkable layer comprising an infrared-absorptive dye that absorbs an infrared light to generate heat, a latent Brønsted acid or s-triazine compound as an acid generator, a resole resin as a crosslinking agent, and a novolak resin as a binder as well as a polymer to be crosslinked as major components, in which after exposure with an infrared laser, the whole of the plate is heated and then developed with an aqueous alkaline solution to obtain a printing plate, as described in JP-A-7-20629 and JP-A-7-271029.
- (5) A lithographic printing plate precursor capable of performing so-called development on printing press comprising a light-sensitive layer having fine particles of a thermoplastic hydrophobic polymer dispersed in a hydrophilic resin provided on a hydrophilic support, which is exposed to an infrared laser, thereby uniting (fusing) the

16

fine particles of thermoplastic hydrophobic polymer by heat to form images, and is mounted on a printing press as it is, followed by supplying damping water and/or ink to remove non-image areas on the printing press, as described in Japanese Patent 2,938,397.

- (6) A printing plate precursor of a type in which a hydrophilic layer containing a colloid such as silica is provided on an oleophilic layer, and the hydrophilic layer is subjected to ablation, as described, for example, in WO94/18005, WO98/40212, and WO99/19143; and a heat-sensitive lithographic printing plate precursor of a type of development on printing press, in which a water-soluble or hydrophilic overcoat layer is provided on a hydrophilic layer in order to prevent scattering of ablation scum, as described in JP-A-2001-96936 and JP-A-2002-86946.
- (7) A lithographic printing plate precursor capable of performing so-called development on printing press comprising a light-sensitive layer having microcapsules encapsulating reactive compounds dispersed therein provided on a hydrophilic support, which is exposed to an infrared laser, thereby collapsing the microcapsules and causing reaction of the reactive compounds to form images, and is mounted on a printing press as it is, followed by supplying damping water and/or ink to remove the non-image areas on the printing press, as described in JP-A-2001-277740, JP-A-2002-137562 and JP-A-2002-46361.

Though the printout element using the heat decomposable dye according to the invention is preferably applied to the lithographic printing plate precursors as described above, it can be applied to lithographic printing plate precursors of any image-forming method so far as they can be adapted for drawing images by heat or heat mode exposure, and it is not limited to the above-described specific examples.

The heat decomposable dye that is used in the invention can be contained in an image-forming layer of the lithographic printing plate precursor. In the case where the lithographic printing plate precursor has a plurality of coating layers, the heat decomposable dye may be contained in other layers than the image-forming layer, such as an ink-accepting layer and an overcoat layer.

A content of the heat decomposable dye that is used in the invention is preferably 1% or more, and more preferably 3% or more based on the total solid content of the layer containing the heat decomposable dye. Good printout images are obtained within such a range.

In the lithographic printing plate precursor of the invention, in order to achieve high sensitization, it is preferred that a light-heat converting agent is contained in the layer containing the heat decomposable dye or a layer adjacent thereto. As the light-heat converting agent, substances absorbing infrared light, particularly near infrared light (wavelength: from 700 to 2,000 nm) are employable, and various pigments, dyes and fine metal particles can be used. For example, the pigments, dyes and fine metal particles as described in JP-A-2001-162960, JP-A-11-235883, *Journal of Japanese Society of Printing Science and Technology*, Vol. 38, pp. 35-40 (2001), and JP-A-2001-213062 are preferably used.

As the pigment, carbon black is particularly preferable. As the fine metal particles are employable fine particles of single metals or alloys selected from Si, Al, Ti, V, Cr, Mn, Fe, Co, Ni, Cu, Zn, Y, Zr, Mo, Ag, Au, Pt, Pd, Rh, In, Sn, W, Te, Pb, Ge, Re, and Sb, or oxides or sulfides thereof. Of these are preferable Re, Sb, Te, Au, Ag, Cu, Ge, Pb, and Sn, with Ag, Au, Cu, Sb, Ge, and Pb being particularly preferred. As the dye are particularly preferable water-soluble group-containing dyes as enumerated below. However, the dye is not limited thereto.



-continued

(IR-7)



(IR-8)



(IR-9)



(IR-10)



(IR-11)



**21**

In the case where the light-heat converting agent is added, e.g., to the oleophilic ink-accepting layer or the polymer fine

**22**

particles, more oleophilic dyes are preferable. Preferred examples of such dyes are illustrated below:

(IR-21)



(IR-22)



(IR-23)



(IR-24)



(IR-25)



(IR-26)



-continued

(IR-27)

 $M = VO$ ,  $R = i-C_5H_{11}$ 

(IR-28)



A content of the pigment or dye as the light-heat converting agent is preferably from 0.1 to 50%, and more preferably from 3 to 40% based on the solid content of the layer containing the pigment or dye. In the case where the fine metal particles are used as the light-heat converting agent, a content of the fine metal particles is preferably 5% or more, and more preferably 10% or more based on the solid content of the layer containing the fine metal particles. Good sensitivity is obtained within such a range.

The support that is used in the invention is a substrate having a hydrophilic surface, or a substrate to which is provided a hydrophilic surface, for example, by applying a hydrophilic layer. Specific examples include paper, paper laminated with plastics (such as polyethylene, polypropylene, and polystyrene), metal sheet (such as aluminum, zinc, and copper), plastic film (such as cellulose diacetate, cellulose triacetate, cellulose propionate, cellulose butyrate, cellulose acetate butyrate, cellulose nitrate, polyethylene terephthalate, polyethylene, polystyrene, polypropylene, polycarbonate, and polyvinyl acetal), paper or plastic film laminated or vapor deposited with the above-described metal, and those substrates having a hydrophilic layer applied thereon. Of these are particularly preferable an aluminum sheet and a polyester film having a hydrophilic layer applied thereon as the support.

As the aluminum sheet, a pure aluminum sheet, and alloy sheet comprised of aluminum as a major component and containing trace amounts of foreign elements can be used. Also, sheet comprising an aluminum or aluminum alloy thin film having a plastic layer laminated thereon can be used.

Examples of the foreign element contained in the aluminum alloy include silicon, iron, manganese, copper, magnesium, chromium, zinc, bismuth, nickel, and titanium. A content of the foreign element in the alloy is at most 10%. An aluminum sheet prepared from an aluminum ingot by the DC casting process and an aluminum sheet prepared from an ingot by the continuous casting process can be used. As the aluminum sheet for use in the invention, aluminum sheets of conventionally known and used materials can be appropriately utilized.

A thickness of the support used in the invention is from 0.05 mm to 0.6 mm, preferably from 0.1 mm to 0.4 mm, and particularly preferably from 0.15 mm to 0.3 mm.

Prior to the use of aluminum sheet, it is preferred to subject the surface of the aluminum sheet to a surface processing such as roughening and anodic oxidation. By the surface processing, not only the hydrophilicity increases, but also it becomes easy to ensure the adhesion to the image-forming layer.

The roughening processing of the surface of aluminum sheet is carried out by various methods. Examples include a method for mechanical roughening, a method in which the surface is electrochemically dissolved and roughened, and a method in which the surface is chemically selectively dissolved. As the mechanical method are employable known methods such as a ball graining method, a brush graining method, a blast graining method, and a buff graining method. As the chemical method, a method in which the aluminum sheet is dipped in a saturated aqueous solution of

an aluminum salt of mineral acid, as described in JP-A-54-31187, is suitable. Further, as the electrochemical roughening method, there is a method in which the aluminum sheet is processed in an electrolytic liquid containing an acid such as hydrochloric acid or nitric acid by an alternating current or a direct current. Moreover, an electrolytic roughening method using a mixed acid, as disclosed in JP-A-54-63902, can be utilized.

Preferably, the roughening by the above-described methods is carried out within the range such that centerline average roughness ( $R_a$ ) of the surface of the aluminum sheet is from 0.2 to 1.0  $\mu\text{m}$ .

If desired, the roughened aluminum sheet is subjected to an alkaline etching processing using an aqueous solution of potassium hydroxide or sodium hydroxide and further subjected to a neutralization processing, and then, if desired, subjected to an anodic oxidation processing in order to enhance abrasion resistance.

As an electrolyte that is used for the anodic oxidation processing of aluminum sheet, various electrolytes for forming a porous oxidized film can be used. In general, sulfuric acid, hydrochloric acid, oxalic acid, chromic acid, and a mixed acid thereof are used. A concentration of the electrolyte is appropriately determined depending on the type of the electrolyte.

The processing conditions of the anodic oxidation vary depending on the electrolyte to be used, and hence, cannot be unequivocally defined. In general, it is suitable that a concentration of the electrolyte in the electrolytic liquid is from 1 to 80%; a liquid temperature is from 5 to 70 °C.; a current density is from 5 to 60 A/dm<sup>2</sup>; a voltage is from 1 to 100V; and an electrolysis time is from 10 seconds to 5 minutes. An amount of the oxidized film formed is preferably from 1.0 to 5.0 g/m<sup>2</sup>, and particularly preferably from 1.5 to 4.0 g/m<sup>2</sup>.

With respect to the support used in the invention, the surface-processed substrate having an anodically oxidized film as described above may be used as it is. But, in order to more improve the adhesion to an upper layer, the hydrophilicity, the anti-staining resistance, the heat insulation, and other properties, if desired, there may be appropriately applied an enlargement process of micro-pores of the anodically oxidized film, a pore-sealing processing of micro-pores, and a surface-hydrophilization processing by dipping in an aqueous solution of a hydrophilic compound, as described in JP-A-2001-253181 and JP-A-2001-322365.

Examples of the hydrophilic compound suitable for the hydrophilization processing include polyvinylphosphonic acid, sulfonic acid group-containing compound, saccharide, citric acid, alkali metal silicate, potassium fluoroziirconate, and phosphate/inorganic fluorine compound.

With respect to the support to be used in the invention, in the case where the hydrophilicity of the surface is insufficient as in a polyester film, it is necessary to render the surface hydrophilic, for example, by applying a hydrophilic layer. As the hydrophilic layer are preferable hydrophilic layers prepared by applying a coating liquid containing a colloid of an oxide or hydroxide of at least one element selected from beryllium, magnesium, aluminum, silicon, titanium, boron, germanium, tin, zirconium, iron, vanadium, antimony, and transition metals, as described in JP-A-2001-199175. Of these are particularly preferable hydrophilic layers prepared by applying a coating liquid containing a colloid of an oxide or hydroxide of silicon.

In the invention, prior to applying the image-forming layer, if desired, may be provided an inorganic undercoat

layer containing, for example, a water-soluble metal salt such as zinc borate, or an organic undercoat layer containing, for example, carboxymethyl cellulose, dextrin, or polyacrylic acid, as described in JP-A-2001-322365. The undercoat layer may contain the above-described light-heat converting agent.

In the lithographic printing plate precursor of the invention, an image is formed by heat or heat mode exposure. Specifically, direct imagewise recording, for example, by a thermal recording head, scanning exposure by an infrared laser, high-illumination flash exposure, for example, by a xenon discharge lamp, and infrared lamp exposure can be used. Exposure by a solid high-output infrared laser such as a semiconductor laser or YAG laser, which radiates near infrared light having a wavelength of from 700 to 1,200 nm is preferred.

The lithographic printing plate precursor of the invention can be irradiated with a laser having a laser output of from 0.1 to 300 W. Further, in the case where a pulse laser is used, it is preferred to irradiate a laser having a peak output of not less than 1,000 W, and preferably not less than 2,000 W. In such a case, an exposure amount falls within a range such that surface exposure intensity before modulation with printing images is preferably from 0.1 to 10 J/cm<sup>2</sup>, and more preferably from 0.3 to 1 J/cm<sup>2</sup>. In the case where the support is transparent, the exposure can be conducted through the support from the backside of the support.

The invention will be described in detail with reference to the following Examples, but the invention should not be construed as being limited thereto.

#### <Preparation of Support>

A melt of an alloy of JIS-A1050, containing 99.5% or more of aluminum, 0.30% of Fe, 0.10% of Si, 0.02% of Ti, and 0.013% Cu, was subjected to a cleaning processing and then cast. In the cleaning processing, in order to remove undesirable gas in the melt, such as hydrogen, a degassing processing was carried out, and a processing with a ceramic tube filter was carried out. The casting was carried out by a DC casting process. A solidified ingot having a plate thickness of 500 mm was subjected to scraping at a depth of 10 mm from the surface, and then to a homogenization processing at 550 °C. for 10 hours such that the intermetallic compounds did not become coarse. Next, the thus processed ingot was subjected to hot rolling at 400 °C. and then to intermediate annealing at 500 °C. for 60 seconds in a continuous annealing furnace, followed by cold rolling to obtain a rolled aluminum sheet having a sheet thickness of 0.30 mm. The roughness of the rolled aluminum sheet was controlled so as to have centerline average roughness ( $R_a$ ) of 0.2  $\mu\text{m}$  after the cold rolling. Thereafter, in order to improve the levelness, the aluminum sheet was made to pass through a tension leveler.

Then, in order to prepare a support for lithographic printing plate, the aluminum sheet was subjected to a surface processing. First, in order to remove rolling oil on the surface of the aluminum sheet, the aluminum sheet was degreased with a 10% sodium aluminate aqueous solution at 50 °C. for 30 seconds and neutralized with a 30% sulfuric acid aqueous solution at 50 °C. for 30 seconds to remove smuts. Next, in order to improve adhesion of a heat-sensitive layer to the support and impart water retention to non-image areas, the aluminum sheet was subjected to a so-called graining to roughen the surface of the support. Specifically, the aluminum web was transported in an aqueous solution containing 1% of nitric acid and 0.5% of aluminum nitrate kept at 45 °C. and subjected to electrolytic graining while giving a current amount at an anode side of 240 C/dm<sup>2</sup> with

an alternating waveform having a duty ratio of 1:1 at a current density of 20 A/dm<sup>2</sup> by an indirect electric supply cell. Thereafter, the aluminum sheet was subjected to an etching processing in a 10% sodium aluminate aqueous solution at 50° C. for 30 seconds and neutralized with a 30% sulfuric acid aqueous solution at 50° C. for 30 seconds to remove smuts.

Further, in order to improve abrasion resistance, chemical resistance, and water retention, an oxidized film was formed on the support by anodic oxidation. Specifically, the aluminum web was transported in a 20% sulfuric acid aqueous solution as an electrolyte at 35° C. and subjected to electrolysis at a direct current of 14 A/dm<sup>2</sup> by an indirect electric supply cell to prepare an anodized film of 2.5 g/m<sup>2</sup>.

Thereafter, in order to ensure hydrophilicity of the non-image areas of printing plate, the support was subjected to a silicate processing. Specifically, the aluminum web was transported in a 1.5% No. 3 sodium silicate aqueous solution kept at 70° C. for a contact time of 15 seconds, and then washed with water. A deposition amount of Si was 10 mg/m<sup>2</sup>. The thus processed support had centerline average roughness (Ra) of 0.25 μm.

<Preparation of Lithographic Printing Plate Precursor (1)>

To the support prepared above was applied an image-forming layer coating solution (A) as prepared below, followed by drying at 80° C. for 3 minutes to prepare a lithographic printing plate precursor (1). A coating amount of the image-forming layer after drying was 1.0 g/m<sup>2</sup>.

Image-forming layer coating solution (A):

|                                                                                                                                                        |         |
|--------------------------------------------------------------------------------------------------------------------------------------------------------|---------|
| Positive type polarity-converting polymeric compound shown below                                                                                       | 0.450 g |
| Light-heat converting agent (IR-24) described above                                                                                                    | 0.025 g |
| Heat decomposable dye (1) described above<br>(Heat decomposition initiation temperature: 220° C., absorption maximum wavelength: 553 nm (in methanol)) | 0.025 g |
| Methyl ethyl ketone                                                                                                                                    | 3.000 g |
| Acetonitrile                                                                                                                                           | 3.000 g |

Positive Type Polarity-Converting Polymeric Compound



<Preparation of Lithographic Printing Plate Precursor (2)>

To the support prepared above was applied an image-forming layer coating solution (B) as prepared below, followed by drying at 80° C. for 3 minutes to prepare a lithographic printing plate precursor (2). A coating amount of the image-forming layer after drying was 1.2 g/m<sup>2</sup>.

Image-forming layer coating solution (B):

|                                                                                                                   |        |
|-------------------------------------------------------------------------------------------------------------------|--------|
| m, p-Cresol novolak (m/p ratio: 6/4, weight average molecular weight: 3,500, containing 0.5% of unreacted cresol) | 1.00 g |
|-------------------------------------------------------------------------------------------------------------------|--------|

-continued

Image-forming layer coating solution (B):

|                                                                                     |        |
|-------------------------------------------------------------------------------------|--------|
| Light-heat converting agent (IR-26) as described above                              | 0.20 g |
| Heat decomposable dye (1) as described above                                        | 0.05 g |
| Fluorine-based surfactant (Megafac F-177 made by Dainippon Ink and Chemicals, Inc.) | 0.05 g |
| γ-Butyrolactone                                                                     | 3.00 g |
| Methyl ethyl ketone                                                                 | 8.00 g |
| 1-Methoxy-2-propanol                                                                | 7.00 g |

<Preparation of Lithographic Printing Plate Precursor (3)>

15 To the support prepared above was applied an image-forming layer coating solution (C) as prepared below, followed by drying at 80° C. for 3 minutes to prepare a lithographic printing plate precursor (3). A coating amount of the image-forming layer after drying was 1.2 g/m<sup>2</sup>.

Image-forming layer coating solution (C):

|                                                                  |         |
|------------------------------------------------------------------|---------|
| Negative type polarity-converting polymeric compound shown below | 1.00 g  |
| Light-heat converting agent (IR-27) described above              | 0.15 g  |
| Heat decomposable dye (1) described above                        | 0.08 g  |
| Fluorine-based surfactant (Megafac F-177)                        | 0.05 g  |
| Methyl ethyl ketone                                              | 20.00 g |
| Methanol                                                         | 7.00 g  |

Negative Type Polarity-Converting Polymeric Compound



45

<Preparation of Lithographic Printing Plate Precursor (4)>

50 To the support prepared above was applied an image-forming layer coating solution (D) as prepared below, followed by drying at 80° C. for 3 minutes to prepare a lithographic printing plate precursor (4). A coating amount of the image-forming layer after drying was 1.5 g/m<sup>2</sup>.

Image-forming layer coating solution (D):

|                                                                                                                                                  |        |
|--------------------------------------------------------------------------------------------------------------------------------------------------|--------|
| Novolak resin obtained from phenol and formaldehyde (alkaline aqueous solution-soluble resin having a weight average molecular weight of 10,000) | 1.5 g  |
| Light-heat converting agent (IR-24) described above                                                                                              | 0.1 g  |
| Heat decomposable dye (1) as described above                                                                                                     | 0.1 g  |
| Acid generating agent (a) shown below                                                                                                            | 0.5 g  |
| Crosslinking agent (b) shown below                                                                                                               | 0.15 g |
| Fluorine-based surfactant (Megafac F-177)                                                                                                        | 0.03 g |
| Methyl ethyl ketone                                                                                                                              | 15 g   |
| 1-Methoxy-2-propanol                                                                                                                             | 10 g   |
| Methanol                                                                                                                                         | 5 g    |



(a)

| Ink-accepting layer coating solution: |                                                                  |        |
|---------------------------------------|------------------------------------------------------------------|--------|
| 5                                     | Epikote 1009 (epoxy resin made by Japan Epoxy Resins Co., Ltd.): | 1.2 g  |
|                                       | Epikote 1001 (epoxy resin made by Japan Epoxy Resins Co., Ltd.): | 0.3 g  |
|                                       | Light-heat converting agent (IR-24) described above              | 0.3 g  |
| 10                                    | Heat decomposable dye (1) described above                        | 0.1 g  |
|                                       | Methyl ethyl ketone:                                             | 13.5 g |
|                                       | Propylene glycol monomethyl ether:                               | 27.0 g |



Then, onto the ink-accepting layer was applied an image-forming layer coating solution (F) as prepared below, followed by drying at 100° C. for one minute to prepare an image-forming layer. A coating amount of the image-forming layer after drying was 0.40 g/m<sup>2</sup>.

| Image-forming layer coating solution (F): |                                                                                                                                                                                     |       |
|-------------------------------------------|-------------------------------------------------------------------------------------------------------------------------------------------------------------------------------------|-------|
| 20                                        | Methanol silica sol (colloid comprising methanol solution containing 30% of silica particles having a particle size of from 10 to 20 nm, made by Nissan Chemical Industries, Ltd.): | 3.0 g |
| 25                                        | Polyacrylic acid (weight average molecular weight: 250,000, made by Wako Pure Chemical Industries, Ltd.):                                                                           | 0.1 g |

Further, an overcoat layer coating solution as prepared below was applied thereto and dried at 100° C. for 1.5 minutes, to form an overcoat layer having a coating amount after drying of 0.15 g/m<sup>2</sup>. Thus, lithographic printing plate precursor (6) was prepared.

| Overcoat layer coating solution: |                                                                                                     |         |
|----------------------------------|-----------------------------------------------------------------------------------------------------|---------|
| 35                               | 28% Aqueous solution of gum arabic                                                                  | 1.5 g   |
|                                  | Light-heat converting agent (IR-10) described above                                                 | 0.042 g |
| 40                               | Emalex #710 (10% aqueous solution made by Nihon Emulsion Co., Ltd.):                                | 0.168 g |
|                                  | Magnesium acetate tetrahydrate (10% aqueous solution, made by Wako Pure Chemical Industries, Ltd.): | 0.03 g  |
|                                  | Distilled water                                                                                     | 30.06 g |

#### <Preparation of Dispersion of Microcapsules>

In a mixture of 12 g of ethyl acetate and 6 g of methyl ethyl ketone were dissolved 6.5 g of adduct of trimethylolpropane and xylene diisocyanate (Takenate D-110N made by Mitsui Takeda Chemicals, Inc.), 2 g of oligomer of diphenylmethane diisocyanate (MR-200 made by Nippon Polyurethane Industry Co., Ltd.), 4 g of a vinyloxy compound shown below, 1.5 g of a light-heat converting agent shown below, 0.5 g of heat decomposable dye (1) described above and 0.1 g of Paionin A-41-C (made by Takemoto Oil & Fat Co., Ltd.) to prepare an oil phase component. As an aqueous phase component, 40 g of a 4% by weight aqueous solution of PVA 205 was prepared. The oil phase component and the aqueous phase component were mixed and emulsified at 12,000 rpm for 10 minutes using a homogenizer. The resulting emulsion was added to 25 g of a 1.5% by weight aqueous solution of tetraethylenepentamine, and the mixture was stirred at room temperature for 30 minutes and then at 65° C. for 3 hours. The microcapsule liquid thus prepared was diluted with distilled water so as to make the solid concentration 20% by weight. The mean particle size of the microcapsules was 0.35 μm. Vinyloxy compound

#### Image-forming layer coating solution (E):

|                                          |        |
|------------------------------------------|--------|
| Dispersion of polystyrene fine particles | 10.0 g |
| Polyacrylic acid                         | 0.12 g |
| Distilled water                          | 10.0 g |

#### <Preparation of Lithographic Printing Plate Precursor (6)>

To the support prepared above was applied an ink-accepting layer coating solution as prepared below, followed by drying at 80° C. for 3 minutes to prepare an ink-accepting layer. A coating amount of the ink-accepting layer after drying was 0.42 g/m<sup>2</sup>.



## Light-Heat Converting Agent



## &lt;Preparation of Lithographic Printing Plate Precursor (7)&gt;

To the support prepared above was applied an image-forming layer coating solution (G) as prepared below, followed by drying at 60° C. for 3 minutes to prepare a lithographic printing plate precursor (7). A coating amount of the image-forming layer after drying was 1.0 g/m<sup>2</sup>.

## Image-forming layer coating solution (G):

|                                                                                                       |        |
|-------------------------------------------------------------------------------------------------------|--------|
| Dispersion of microcapsules                                                                           | 10 g   |
| Acid precursor shown below                                                                            | 0.2 g  |
| Fluorine-based surfactant (Megafac F-171 made by Dainippon Ink and Chemicals, Inc.)                   | 0.05 g |
| Distilled water (in an amount so as to make the solid concentration of coating solution 7% by weight) |        |

## Acid Precursor



## &lt;Preparation of Comparative Lithographic Printing Plate Precursor (1')&gt;

The same procedures as in the preparation of the lithographic printing plate precursor (1) were followed, except for using a coating solution prepared by eliminating the heat decomposable dye from the image-forming layer coating solution (A) used in the preparation of the lithographic printing plate precursor (1) to prepare a comparative lithographic printing plate precursor (1'). A coating amount of the image-forming layer after drying was 0.95 g/m<sup>2</sup>.

## &lt;Preparation of Comparative Lithographic Printing Plate Precursor (2')&gt;

The same procedures as in the preparation of the lithographic printing plate precursor (2) were followed, except for using a coating liquid prepared by eliminating the heat decomposable dye from the image-forming layer coating solution (B) used in the preparation of the lithographic printing plate precursor (2) to prepare a comparative lithographic printing plate precursor (2'). A coating amount of the image-forming layer after drying was 1.1 g/m<sup>2</sup>.

## 10 &lt;Preparation of Comparative Lithographic Printing Plate Precursor (3')&gt;

The same procedures as in the preparation of the lithographic printing plate precursor (3) were followed, except for using a coating liquid prepared by eliminating the heat decomposable dye from the image-forming layer coating solution (C) used in the preparation of the lithographic printing plate precursor (3) to prepare a comparative lithographic printing plate precursor (3'). A coating amount of the image-forming layer after drying was 1.1 g/m<sup>2</sup>.

## 15 &lt;Preparation of Comparative Lithographic Printing Plate Precursor (4')&gt;

The same procedures as in the preparation of the lithographic printing plate precursor (4) were followed, except for using a coating liquid prepared by eliminating the heat decomposable dye from the image-forming layer coating solution (D) used in the preparation of the lithographic printing plate precursor (4) to prepare a comparative lithographic printing plate precursor (4'). A coating amount of the image-forming layer after drying was 1.5 g/m<sup>2</sup>.

## 20 &lt;Preparation of Comparative Lithographic Printing Plate Precursor (5')&gt;

The same procedures as in the preparation of the lithographic printing plate precursor (5) were followed, except for using a dispersion of fine particles prepared by eliminating the heat decomposable dye from the dispersion of polystyrene fine particles used in the preparation of the lithographic printing plate precursor (5) to prepare a comparative lithographic printing plate precursor (5'). A coating amount of the image-forming layer after drying was 0.8 g/m<sup>2</sup>.

## 25 &lt;Preparation of Comparative Lithographic Printing Plate Precursor (6')&gt;

The same procedures as in the preparation of the lithographic printing plate precursor (6) were followed, except for using an ink-accepting layer coating liquid prepared by eliminating the heat decomposable dye from the ink-accepting layer coating solution used in the preparation of the lithographic printing plate precursor (6) to prepare a comparative lithographic printing plate precursor (6'). A coating amount of the ink-accepting layer after drying was 0.42 g/m<sup>2</sup>. A coating amount of the image-forming layer after drying was 0.40 g/m<sup>2</sup>. A coating amount of the overcoat layer after drying was 0.15 g/m<sup>2</sup>.

## 30 &lt;Preparation of Comparative Lithographic Printing Plate Precursor (7')&gt;

The same procedures as in the preparation of the lithographic printing plate precursor (7) were followed, except for using a dispersion of microcapsules prepared by eliminating the heat decomposable dye from the dispersion of microcapsules used in the preparation of the lithographic printing plate precursor (7) to prepare a comparative lithographic printing plate precursor (7'). A coating amount of the image-forming layer after drying was 1.0 g/m<sup>2</sup>.

## EXAMPLES 1 TO 7 AND COMPARATIVE EXAMPLES 1 TO 7

65 Each of the thus prepared lithographic printing plate precursors was installed in Trendsetter 3244VX made by

CreoScitex and irradiated with an energy as described in Table 1 to form latent image. After the exposure, the lithographic printing plate precursor was visually observed, and the printout property was evaluated according to the following criteria: A=good and B=poor. Then, of the precursors each having latent image formed therein, the precursors (1), (3), (5), (6), (7), (1'), (3'), (5') and (7') were mounted as they were without being processed on an SOR-M printing press made by Heidelberg, and subjected to printing in a usual manner. Further, the precursors (2) and (2') each having latent image formed therein were developed by using an automatic processor (PS Processor 900VR made by Fuji Photo Film Co., Ltd.) charged with a developing solution (DP-4 made by Fuji Photo Film Co., Ltd.) and a rinsing solution (FR-3 made by Fuji Photo Film Co., Ltd.) (1:7), and then subjected to printing in the same manner as described above. Moreover, the precursors (4) and (4') each having latent image formed therein were heated in an oven at 140° C. for one minute, and then developed and subjected to printing in the same manner as in the precursors (2) and (2'). The results obtained are set forth in Table 1.

TABLE 1

Examples 1 to 7 and Comparative Examples 1 to 7

|                       | Lithographic Printing Plate Precursor | Exposure Energy (mJ/cm <sup>2</sup> ) | Printout Property | Number of Prints (x10,000) |
|-----------------------|---------------------------------------|---------------------------------------|-------------------|----------------------------|
| Example 1             | (1)                                   | 400                                   | A                 | 5                          |
| Example 2             | (2)                                   | 150                                   | A                 | 8                          |
| Example 3             | (3)                                   | 400                                   | A                 | 4                          |
| Example 4             | (4)                                   | 200                                   | A                 | 10                         |
| Example 5             | (5)                                   | 250                                   | A                 | 2                          |
| Example 6             | (6)                                   | 240                                   | A                 | 2                          |
| Example 7             | (7)                                   | 400                                   | A                 | 4                          |
| Comparative Example 1 | (1')                                  | 400                                   | B                 | 5                          |
| Comparative Example 2 | (2')                                  | 150                                   | B                 | 8                          |
| Comparative Example 3 | (3')                                  | 400                                   | B                 | 4                          |
| Comparative Example 4 | (4')                                  | 200                                   | B                 | 10                         |
| Comparative Example 5 | (5')                                  | 250                                   | B                 | 2                          |
| Comparative Example 6 | (6')                                  | 240                                   | B                 | 2                          |
| Comparative Example 7 | (7')                                  | 400                                   | B                 | 4                          |

From the results shown in Table 1, it can be seen that in any of the lithographic printing plate precursors of the Examples, the printout property was good, and the drawn images could be clearly confirmed. On the other hand, in any of the comparative lithographic printing plate precursors not containing the heat decomposable dye, the printout property was poor, and it was difficult to distinctly confirm the drawn images. In addition, all of the lithographic printing plate precursors of the Examples and Comparative Examples had equivalent sensitivity and printing durability, and thus influences against other printing performances brought by the addition of heat decomposable dye were not observed.

According to the invention, a lithographic printing plate precursor having good printout property, which is capable of drawing images by heat or heat mode exposure, can be obtained.

The entire disclosure of each and every foreign patent application from which the benefit of foreign priority has been claimed in the present application is incorporated herein by reference, as if fully set forth herein.

While the invention has been described in detail and with reference to specific embodiments thereof, it will be apparent to one skilled in the art that various changes and modifications can be made therein without departing from the spirit and scope thereof.

What is claimed is:

1. A lithographic printing plate precursor having an image-forming layer capable of forming images by heat or heat mode exposure and development with an aqueous 10 alkaline solution, which comprises a support and a layer containing a heat decomposable dye having an absorption maximum wavelength in a visible region, not substantially having an absorption in an oscillation wavelength of a laser used for heat mode exposure, and having a heat decomposition initiation temperature of 250° C. or lower.

15 2. The lithographic printing plate precursor as claimed in claim 1, wherein the heat decomposable dye has a structure represented by the following formula (1) or (2):



30 wherein A, A', B, and B' each independently represents a substituent; Y and Z each represents an atomic group necessary for forming a carbon ring or a heterocyclic ring; E and G each represents an atomic group to complete a conjugated double bond chain; X and X' each represents oxygen, N-R, or C(CN)<sub>2</sub>; R represents an alkyl group or an aryl group; L<sup>3</sup>, L<sup>4</sup>, L<sup>5</sup>, L<sup>6</sup>, and L<sup>7</sup> each represents a methine group which may be substituted; M<sup>k+</sup> represents an onium ion; m and n each independently represents 0, 1, or 2; x and y each independently represents 0 or 1; and k represents an integer of 1 or more.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 916

## 35

7. The lithographic printing plate precursor as claimed in claim 2, wherein the heat decomposable dye has a structure represented by the following formula (1) or (2):



8. The lithographic printing plate precursor as claimed in claim 6, wherein the image-forming layer comprises a hydrophobic polymer compound that can be rendered hydro-

## 36

philic by heat and has a functional group selected from a sulfonic ester group, a sulfonimido group and a disulfone group.

9. The lithographic printing plate precursor as claimed in claim 6, wherein the image-forming layer comprises fine particles of a thermoplastic hydrophobic polymer.

10. The lithographic printing plate precursor as claimed in claim 6, wherein the image-forming layer comprises micro-capsules encapsulating an oleophilic compound.

11. A lithographic printing plate precursor having an image-forming layer capable of drawing images by heat or heat mode exposure, which comprises a support, an oleophilic layer containing a heat decomposable dye having an absorption maximum wavelength in a visible region, not substantially having an absorption in an oscillation wavelength of a laser used for heat mode exposure, and having a heat decomposition initiation temperature of 250° C. or lower, and a hydrophilic layer in this order.

\* \* \* \* \*